

## UNITED STATES PATENT OFFICE

2,421,672

## RUST PREVENTIVE COMPOSITION

Chester E. Wilson, San Pedro, and Mary Louise Dodge, Long Beach, Calif., assignors to Union Oil Company of California, Los Angeles, Calif., a corporation of California

No Drawing. Application January 21, 1944,  
Serial No. 519,202

21 Claims. (Cl. 106—14)

1

This invention relates to compositions having high degrees of efficiency for preventing rusting or corrosion of ferrous and other metal surfaces.

An object of this invention is to produce an anti-rust composition which will protect metals especially iron and steel against corrosion under severe conditions and over prolonged periods of exposure, when applied in thin films.

Another object of the invention is to prepare a rust preventive composition which may be readily applied to metal surfaces and which may be easily removed from such metal surfaces by ordinary solvents even after long periods of exposure to the atmosphere.

A further object of the invention is to prepare a rust preventive composition which will dry in a relatively short time yielding a non-tacky film which is tough and will resist shock and which will also adhere tenaciously to the metal surfaces even under wide extremes of temperature variations.

In its broadest aspects the invention comprises oil-soluble soaps of fats, fatty oils and organic acids capable of adhering tenaciously to metal surfaces in the presence of moisture and under varying temperature conditions after such soaps have been applied as a solution in a thinner, as for example, a light mineral solvent. Such oil-soluble soaps may be typified by a lead soap of tall oil which may be considered to be a semi-drying oil and the lead soap of acids which may be produced by oxidizing hydrocarbons, as for example, by oxidizing paraffin wax or a highly paraffinic lubricating oil fraction or petrolatum. While these soaps may be used separately for best results both of these types of soap are employed. Roughly about one-half of the finished rust preventive composition will be the mixture of soaps, the other half being thinner. Depending upon the purity of the synthetic acids, i. e., their freedom from unoxidized or partially oxidized oil and/or wax we may employ for the purpose of promoting greater water resistance, a few per cent of a low melting point paraffin wax or petrolatum, i. e., from about 1% to perhaps 6%. Similarly, depending upon the purity of the synthetic acids employed, a small percentage of a paraffinic type lubricating oil may be added, e. g., from about 1% to about 6% for the purpose of plasticizing the product and avoiding objectionable brittleness in the applied and dried film. Relatively small proportions of an oil-soluble metal sulfonate may also be included in our rust preventive composition. The sulfonate has the effect of furnishing increased protection against corrosion and it re-

duces materially the pour point of the finished composition.

The term "oil-soluble" as used herein is meant to include good dispersibility or colloidal distribution in oil and not necessarily true solution.

In addition to the above indicated ingredients and in order to secure an important object of the invention, that is drying to a non-tacky film in a comparatively short period of time, a small proportion of an active drier is employed. Driers which are found to be particularly effective for this purpose are oil-soluble cobalt salts, i. e., cobalt naphthenate, linoleate, tall oil soap, or the like, or in some cases the corresponding manganese salts may be employed. For practical purposes the finished rust preventive composition should contain in the order of about 0.01% of cobalt calculated as the metal where about one-half of the composition is thinner.

20 One very desirable composition contained the following:

|                                       | Approximate Per Cent by Weight |                 |
|---------------------------------------|--------------------------------|-----------------|
|                                       | With Thinner                   | Without Thinner |
| 25                                    |                                |                 |
| Lead Soap of Tall Oil                 | 38.0                           | 69              |
| Lead Soap of Wax Oxidate <sup>1</sup> | 12.0                           | 22              |
| Sodium Sulfonate <sup>2</sup>         | 5.0                            | 9               |
| Cobalt Drier (as metal)               | 0.01                           | 0.02            |
| Petroleum Thinner                     | 45.0                           | None            |

<sup>1</sup> This wax oxidate was prepared by oxidizing a paraffin wax (122° F. to 125° F. M. P.) for a period of 50 hours at 250° F. and at normal atmospheric pressure, in the presence of 0.5% manganese naphthenate catalyst, the oxidate had an acid number of 105 mg. KOH/g. and a saponification number of 210 mg. KOH/g.

<sup>2</sup> The sodium salt of oil-soluble (mahogany) sulfonic acids.

Another very desirable composition contained the following:

|                                         | Approximate Per Cent by Weight |                 |
|-----------------------------------------|--------------------------------|-----------------|
|                                         | With Thinner                   | Without Thinner |
| 40                                      |                                |                 |
| Lead Soap of Tall Oil                   | 34.0                           | 60              |
| Lead Soap of Wax Acids <sup>1</sup>     | 15.0                           | 26              |
| Paraffin Wax (122° F. to 125° F. M. P.) | 4.0                            | 7               |
| Lubricating Oil                         | 4.0                            | 7               |
| Cobalt Drier (as metal)                 | 0.01                           | 0.02            |
| Petroleum Thinner                       | 43.0                           | None            |

<sup>1</sup> The wax acids were obtained from the wax oxidate used in the first composition noted above by saponifying said oxidate with aqueous NaOH, separating the aqueous sodium soap phase from the unsaponifiable phase and freeing the acids from the soap phase by acidifying with dilute mineral acid.

55 The proportions of the various components of

the above rust preventive compositions may be modified, the components themselves may be substituted for by other similar materials as indicated hereinbelow, or various constituents may be entirely omitted according to the characteristics required in a given product for a given use. The effect of composition upon the characteristics of the resultant rust preventive film is briefly discussed herebelow.

If the composition consists wholly of thinner and oil-soluble lead tall oil soap or oil-soluble soap of another semi-drying oil, the product would be hard and brittle when dried and, moreover would not be readily removable by ordinary solvents after a few months of exposure and therefore the product would not be satisfactory for most uses. Similarly, if the proportion of tall oil soap with respect to other constituents is too great, the dried product becomes too brittle. Again, if the oil-soluble metal soap of synthetic acids is the only constituent employed with the thinner the resulting dried film is too soft and the viscosity and pour point of the solvent or thinner solution of this soap are too high, making its application to metal surfaces needlessly difficult. If, however, from about 5% to about 30% of the oil-soluble metal soap of synthetic acids, based on the non-volatile constituents, is used the product remains readily removable after long periods of exposure. Around 5% of the synthetic acid soap (based on the non-volatile constituents) appears to be the minimum necessary to insure ready removal of the resultant rust preventive film after several weeks or months of exposure.

The most desirable proportion of oil-soluble metal soap of synthetic acids in a finished rust preventive composition is between about 10% and about 40% by weight of the non-volatile constituents or between about 5% and about 20% by weight of the thinned composition. However, we may use between about 3% and about 85% by weight of this soap based on the non-volatile constituents and, correspondingly, between about 1.5% and about 42.5% by weight based on the thinned product. Similarly, we prefer to use between about 50% and about 90% by weight of an oil-soluble metal soap of a semi-drying oil, based on the non-volatile constituents, or between about 25% and about 45% by weight based on the thinned product. However, we may use between about 5% and about 95% based on the non-volatile constituents or between about 2.5% and 47.5% based on the thinned product.

Although the relative brittleness or tackiness of the applied and dried film may be controlled as indicated above, i. e., by varying the proportion of the two types of soaps employed, an additional and desirable means of controlling brittleness of the applied film as well as viscosity and particularly pour point of a thinned rust preventive composition is to include in the rust preventive composition small percentages of a metal sulfonate, such as an alkali or alkaline earth or heavy metal salt of sulfonic acids obtained by sulfonating petroleum hydrocarbons. Thus metals such as sodium, potassium, lithium, calcium, barium, strontium, magnesium, lead, zinc, etc., all produce sulfonates which may be used in our composition. Such sulfonates when employed in concentrations ranging from about 1% to about 5% or even as high as 10% by weight of the thinned rust preventive have the effect of reducing the pour point and the apparent viscosity of the thinned product. Moreover, rust preventive

compositions containing such sulfonates give even better protection against corrosion when applied to metal surfaces. Sulfonates which have been found to be particularly desirable include the sodium, barium, and lead salts of oil-soluble sulfonic acids produced by concentrated or fuming sulfuric acid treatment of lubricating oils. These oil-soluble sulfonic acids are usually referred to as mahogany acids. In those instances in which the indicated sulfonates are used the proportion of the oil-soluble soaps of synthetic acids may be correspondingly reduced or the sulfonates may be substituted for a portion or all of the lubricating oil which otherwise may be employed since the sulfonates have a plasticizing action on the resultant dried film.

The paraffin wax is employed to render the composition more water resistant. This paraffin wax may be added as such, or in those instances in which a wax oxidate is employed for the preparation of the lead soaps of synthetic acids, there may be sufficient paraffin wax or non-acidic partially oxidized paraffin wax present in the oxidate to impart the desired water resistance to the finished composition. In those cases in which the synthetic acids are separated from the wax oxidate before being converted into a usable oil-soluble soap such as a lead soap it may be desirable to add small proportions of paraffin wax to the composition. Also in those cases in which the synthetic acids are produced by oxidizing highly paraffinic oils whether the acids are first purified or not, it may be desirable to include small proportions of paraffin wax in the composition. While the wax is employed to render the composition more water resistant it has the effect of producing a dull finish in the rust preventive film which eliminates light reflections from treated surfaces. This effect appears to be due to a slight incompatibility of the wax. When 2% to 3% or less of the total composition, i. e., including thinner, is paraffin wax the product is still very desirable but the finish when dry tends to be shiny. If the proportion of paraffin wax is increased above about 4% the pour point of the rust preventive solution in thinner is raised to an objectionable degree. Thus the 4% of paraffin wax based on the thinned product approaches the critical concentration. We prefer to use, therefore, up to about 8% or 9% by weight of paraffin wax based on the non-volatile constituents and we may use as much as about 12% by weight of wax. The amount to be employed in any given case will, as indicated hereinabove, depend upon the utilization of the product and upon the purity, i. e., the freedom from wax and/or oil of the synthetic acids used in its preparation.

In place of the paraffin wax we may use petro-  
60 latum which is a micro-crystalline or amorphous wax obtained by dewaxing paraffinic residual oils. The proportion of petrodatum which may be successfully employed is somewhat higher than the limits indicated for paraffin wax because the  
65 petrodatum does not raise the pour point of the thinned rust preventive composition to as great an extent as does the paraffin wax. Thus we may use up to about 15% by weight of petrodatum based on the non-volatile constituents although  
70 amounts less than about 10% by weight are generally more desirable. The amount to be employed in any given case will depend upon the purity of the synthetic acids employed in the composition.

75 The lubricating oil is employed to plasticize the

composition and make the dried rust preventive film less brittle. Preferably the lubricating oil should be rather heavy, such as one having a viscosity of 150 seconds Saybolt Universal at 210° F. corresponding with 70 SAE grade. Here again about 4% of oil based on the total composition approaches the critical, inasmuch as larger proportions of lubricating oil tend to retard the drying excessively and tend to make the dried film too soft. As in the case of the paraffin wax or the petrolatum, the amount of lubricating oil used will depend upon the character of synthetic acids, i. e., whether they were prepared from a highly paraffinic oil fraction or whether they were prepared from a paraffin wax, and also upon the degree of purity of the synthetic acids, i. e., whether they were separated from unsaponifiable components present in the oxidate. Thus, if a paraffinic oil oxidate were converted into the lead or other oil-soluble metal soap the purified rust preventive compositions prepared from such lead soaps, would be sufficiently plastic in most instances without the addition of further quantities of lubricating oil. On the other hand, if the paraffinic oil oxidate was first separated into an acid fraction and a fraction comprising the unsaponifiable components and the thus separated acids converted into lead soaps it would usually be desirable to include small proportions of lubricating oil or its equivalent in rust preventive compositions containing these soaps. Thus it will be seen that we may prefer to use up to about 8% by weight of lubricating oil based on the non-volatile constituents, however, we may use as high as about 12% by weight of oil.

The amount of cobalt drier previously indicated, i. e., 0.01% based on the finished composition, is within the practical limits. If much less drier is used its effectiveness is inconsequential, and if greater proportions than about 0.1% (metal content in thinned product) are employed no appreciable additional benefits appear to be obtained. The presence of the drier speeds up the drying of the applied film so that good drying may be obtained in as little as six to eight hours. If the time of drying is of no consequence, so that a drying period of twenty to fifty hours or more is not objectionable, the drier may be eliminated. On the other hand, if drying within two or three hours is required, the cobalt content of the finished rust preventive may be increased to two or three times the indicated 0.01%. The use of greater proportions than 0.1% is in no way objectionable and amounts as large as 0.2% or even 0.3% of cobalt in the form of cobalt drier may be employed in certain instances.

In those cases in which extremely active drier metals, e. g., cobalt or manganese are used in the rust preventive composition in the form of soaps of either the synthetic acids or the semi-drying oils, it is usually not necessary to add additional drier. When less active drier metals, such as lead, zinc, etc., are employed the cobalt or other drier is to be used when rapid drying of the applied film is desired.

Although in general we prefer to use about 50% by weight of an ordinary petroleum thinner, as indicated hereinabove, the proportion of thinner may be varied depending upon the use for which the rust preventive is intended. Desirable rust preventives have been prepared containing as little as about 30% by weight of thinner and as high as about 70% by weight of thinner based upon the total composition. The thinner may be any readily volatile mineral oil fraction such

as mineral spirits or naphtha or equivalent thinner.

In some instances, particularly in those cases in which it is desirable that the finished rust preventive composition have a flash point above about 100° F. the thinner selected may be one having a flash point slightly above the indicated value. In such cases it is preferable that the high flash point thinner have a relatively narrow boiling point range in order to avoid the presence of high boiling components which if present would retard the drying of the applied rust preventive film. Such a thinner would be a petroleum naphtha having a boiling point range of about 310° F. to about 375° F. or even as high as 400° F.

#### *Semi-drying oils and/or acids*

The tall oil which is converted into an oil-soluble metal soap to produce one component of our rust preventive composition may, for the purposes of this application, be considered to be a semi-drying oil. Tall oil which consists chiefly of resin acids, fatty acids and unsaponifiable material is a by-product of wood pulp manufacture and is well known in commerce. We may use the unrefined tall oil or the refined tall oil depending upon the use to which the finished anti-rust composition is to be placed. Thus if a relatively light colored rust preventive film is desirable we may use a refined or a distilled tall oil, however, in those cases in which appearance is not important, we may prefer to use the unrefined tall oil.

Other oils which are generally classified as semi-drying oil may be employed in place of all or part of the tall oil in any given case. Thus we may use an oil-soluble metal soap of rape seed oil, cotton seed oil, corn oil, rice oil, colza oil, mustard seed oil, sesame oil and like oils in place of the oil-soluble metal soap of tall oil. In those instances in which one of the last named group of semi-drying oils is used to replace all of the tall oil, the proportion of the oil-soluble metal soap of this oil will usually be reduced somewhat from the amount of oil-soluble metal soap of tall oil employed and the oil-soluble metal soap of synthetic acids will be correspondingly increased because most of these semi-drying oils produce a harder film and a film that is more difficult to remove after exposure than does tall oil.

In some instances it may be desirable to use an oil-soluble metal soap of a drying oil such as linseed oil, China-wood oil, tung oil and the like. In general it is not desirable to replace all of the tall oil or semi-drying oil with a drying oil, however, rust preventive compositions containing as much as 5% to 10% by weight of an oil-soluble metal soap of a drying oil, based upon the non-volatile constituents, replacing an approximately equal quantity of an oil-soluble metal soap of tall oil have been found to be very good anti-rust agents.

#### *Oil-soluble metal soaps of semi-drying oils and/or acids*

The above semi-drying oils and/or acids may be converted into soaps such as, for example, lead soaps which are the preferred type of soaps, by saponifying the semi-drying oil with sodium hydroxide to produce the sodium soap and then preparing the lead soap from the sodium soap by metathesis. The required quantity of semi-drying oil is charged to a steam jacketed kettle equipped with an agitator and the theoretical

quantity of caustic soda, indicated by the saponification number of the oil, is added in the form of a 10% to 50% NaOH solution in water. With the agitator in motion the batch is heated slowly to the boiling point and held at this temperature until analysis indicates that the reaction is complete and all of the caustic soda has been utilized. If necessary and particularly where concentrated NaOH solutions are used small additions of water may be made during the course of the saponification. It is important that no free caustic shall be present at the completion of the saponification and if necessary, a small addition of fatty oil may be made to neutralize any free caustic soda present after a reasonable heating period. When saponification is complete the charge is diluted with water to yield a soap content of 10% to 20% by weight. To the dilute soap, which should be at a temperature between about 180° F. and 200° F., is added the theoretical quantity of lead acetate in the form of a 25% solution in water. The amount of lead acetate to be added is calculated from the methyl orange soap number of the dilute soap solution. The lead acetate is added as rapidly as it will be taken up by the batch and during the addition the agitator is kept in motion. To complete the formation of the lead soap, the batch is maintained at a temperature of 180° F. to 200° F. for approximately one hour and at this time no more than a small amount of free lead ion should be present as indicated by a test with potassium dichromate solution. The agitator is then stopped and the lead soap of the semi-drying oil is allowed to separate from the aqueous phase. The separated water is drained from the kettle and the lead soap washed with hot water until free from lead ion. The batch is then dehydrated by heating to 325° F. to 340° F. with agitation. When dehydration is complete, thinner may be added at the lowest practical temperature to yield a solution of lead soap containing approximately 50% by weight of the soap.

The soaps may also be prepared by heating the oil with the theoretical quantity of litharge, the proportions of litharge to oil varying with the acid number or the saponification number of the oil and the purity of the litharge. Thus the oil is heated in a steam jacketed kettle equipped with an agitator, and when the temperature of the oil reaches 250° F. to 300° F. the litharge is added slowly. During the addition of litharge or after the addition of litharge has been completed the charge may be blown with steam to increase the rate of reaction. Steam blowing is particularly desirable when fatty oils or other glycerides are employed as the soap stocks. In those cases in which the soap stocks are primarily free acids, e. g., tall oil, the use of steam is not required and care should be taken to prevent excessive foaming during the reaction which may result from the liberation of water. In any case temperatures should be maintained between about 300° F. and about 350° F. until reaction is complete. This will require from one to two hours or even longer in the case of some of the fatty oils. When the reaction is complete, the batch is cooled to about 250° F. and may then be thinned by the gradual addition of a thinner such as a mineral solvent having a boiling range of approximately 315° F. to 380° F. until the resulting solution of soap in thinner contains approximately 50% by weight of soap. The finished batch is held at a temperature of about 100° F. for eighteen to twenty-four hours to permit settling of the unreacted

7  
litharge or other insoluble impurities, and then decanted from the settling and run to storage.

In those cases in which a mixture of semi-drying oils or in which tall oil and one of the other semi-drying oils is to be employed in the rust preventive composition, the oil-soluble metal soap may be prepared from each oil alone or from the mixture of the two oils. Generally the first method of preparation, i. e., the one involving saponification followed by metathesis is preferable for preparing the mixed soaps or for preparing the soaps of any of the glycerides.

In addition to lead, other metals may be employed to form desirable oil-soluble metal soaps. Thus the alkaline earth metals, calcium, barium, strontium, and magnesium, may be employed in place of part or all of the lead in the preparation of the above soaps. We may also use iron, cobalt, manganese, zinc, tin, nickel, chromium, vanadium, copper, and other like heavy metals. A more complete discussion of the metals which may be employed is given hereinbelow.

#### Synthetic organic acids

The second soap component of our rust preventive composition referred to hereinabove as an oil-soluble metal soap of acids produced by the oxidation of paraffin wax, highly paraffinic mineral oil fractions or petrolatum is prepared from the crude oxidate or from acids separated from the crude oxidate. Desirable synthetic acids may be produced from one of the oxidation stocks listed below and in the manner described.

A primary requirement of synthetic organic acids which may be used in our rust preventive composition is that the acids from soaps with the metals disclosed hereinabove which are sufficiently soluble in oil and in mineral solvents or thinners to permit their use in combination with the above described oil-soluble soaps of semi-drying oils in a mineral thinner solution. Since oil solubility of such soaps depends upon the molecular weight of the acids from which they are produced, stocks employed for oxidation must be composed of hydrocarbon molecules having relatively high molecular weights. Hydrocarbon fractions which have been found to be satisfactory oxidation stocks include petroleum waxes such as those normally referred to as paraffin waxes, petrolatums, foots oil, which is a highly paraffinic high pour point oil separated from paraffin waxes during the final stages of their purification by means of cold pressing, etc., and highly paraffinic lubricating oils having viscosities greater than about 40 seconds Saybolt Universal at 210° F. Such paraffinic lubricating oils are those highly solvent treated lubricating oils having viscosity indices of about 85 or above and viscosity gravity constants of about 0.82 or below.

In preparing a satisfactory oxidate from a paraffin wax for example, a pressure vessel is charged with the desired quantity of a paraffin wax having a melting point of about 120° F. and a small quantity, i. e., about 0.75% by weight, based on the paraffin wax, of manganese naphthenates which acts as an oxidation catalyst. The vessel is pressurized to about 100 lbs./sq. in. gage and the wax heated to a temperature of approximately 250° F. Air is introduced into and finely dispersed in the molten wax until the oxidate has an acid number of about 200 mg. KOH/g. requiring between about 35 and 50 hours of treatment depending upon the temperature, pressure, catalyst, etc. This oxidate may be used directly for conversion into the desired metal soap or may be first refined to separate the acidic constituents

contained therein from the non-acidic or unsaponifiable materials.

The method of producing a desirable oxidate is not limited to that described above, for the oxidation has been satisfactorily effected by air-blowing this paraffin wax at ordinary atmospheric pressures and temperatures of about 250° F. in the presence of an oxidation catalyst and in fact in some instances atmospheric pressure oxidation results in the production of a higher grade oxidate than does pressure oxidation. Oxidates produced in this manner and having acid numbers of 100 mg. KOH/g. or above, such as 120 mg. KOH/g. or higher are particularly desirable and have been prepared by air-blowing for periods of 40 to 75 hours. In those cases in which the acid number of the wax oxidate is below about 100 mg. KOH/g. it is usually desirable to separate the acids from the oxidate for if the crude oxidate itself were used the proportion of unoxidized wax carried with the oil-soluble metal soap into the rust preventive composition would be objectionably high.

Lubricating oil such as one disclosed hereinabove may be oxidized by either process described for the oxidation of paraffin wax. In this case, however, the oxidation is preferably continued until the oxidate has an acid number in the order of 40 to 60 mg. KOH/g. although in some instances it may be desirable to produce oil oxidates having acid numbers as high as 100 mg. KOH/g. In those cases in which the acid number of the oil oxidate is below about 50 mg. KOH/g. it is usually desirable to separate the acids from the oxidate before preparing the oil-soluble metal soap of the acids in order to eliminate the rather large proportions of unoxidized oil contained in such low acid number oxidates.

As is well known the controlled partial oxidation of hydrocarbon fractions such as those disclosed above results in the production of alcohols, ketones, esters and other partial oxidation products along with the desired acids. The presence of these partial oxidation products in the soaps prepared from the synthetic acids is in no way undesirable or objectionable, unless, as indicated above, the proportion of unoxidized wax or oil and partial oxidation products is great enough that a dried film, produced by a rust preventive composition containing soaps having the high wax or oil content is too soft. Generally, however, in those cases in which the oxidation is continued until the oxidate has an acid number of about 100 mg. KOH/g. or higher for the wax or about 50 or higher for the oil, the proportion of unoxidized wax or oil and of partial oxidation products other than acids will be sufficiently reduced to permit the use of the oxidate without separating the synthetic acids therefrom.

The oxidation of the paraffin wax and of lubricating oil may be effected without the use of a catalyst. However, in general we prefer to oxidize in the presence of a small proportion, i. e., in the order of from about 0.5% to 1.0% or even as much as 2 to 3% of an oil-soluble salt such as a naphthenate, oleate or like salt of manganese, calcium, magnesium, iron, cobalt or other like polyvalent metal. Manganese is particularly desirable both from the point of view of catalytic activity and the production of light colored oxidates. Iron is a particularly active catalyst for the oxidation, however, oxidates produced using an iron catalyst are usually dark in color and thus may be objectionable in those cases in which light colored rust preventive compositions are desired. On the

other hand, if a dark colored rust preventive is not objectionable iron naphthenate may desirably be used as a catalyst for the oxidation of paraffin wax or lubricating oil because of its extremely active catalytic effect.

#### *Oil-soluble metal soaps of synthetic organic acids*

In preparing oil-soluble metal soaps, as for example, lead soaps of the synthetic organic acids either of the two processes described for preparing oil-soluble metal soaps of semi-drying oils may be employed. Thus the crude oxidate or the crude oxidate after being water washed to remove water-soluble acidic constituents may be treated directly with litharge at temperatures in the order of 250° F. to 300° F. until reaction is complete and the product then cooled and diluted with thinner so that the resulting soap solution contains approximately 50% by weight of soap. According to the second method, the crude oxidate or the water washed crude oxidate is first saponified with the theoretical quantity of sodium hydroxide and the resulting sodium soaps may be converted into lead soaps, for example, by the addition of lead acetate in theoretical quantities. The thus produced lead soaps are separated from the aqueous layer containing sodium acetate, etc., and washed free from lead ion with hot water. The washed soaps are then dehydrated and may be thinned with mineral solvent to produce a solution containing approximately 50% by weight of soap.

In those instances in which it is desired to use a refined or substantially oil- or wax-free synthetic organic acid, the crude oxidate is saponified with sodium hydroxide at temperatures in the order of 300° F. for a period of two to three hours and the saponified mixture allowed to separate into an aqueous sodium soap phase, and an oily phase comprising unoxidized oil and/or wax and non-acidic partial oxidation products. The aqueous soap phase is separated from the oil phase and then treated with the theoretical quantity of lead acetate (25% aqueous solution) to convert the sodium soaps into lead soaps. The thus produced lead soaps are washed free from lead ion by means of hot water, dried by heating and may then be thinned as above with mineral solvent.

Other metals which we may employ in place of lead include those listed hereinabove for preparing oil-soluble soaps of semi-drying oils and these metals are more fully discussed below.

#### *Metals*

The metals which we may use for producing oil-soluble metal soaps of semi-drying oils and of synthetic organic acids may be classified into two groups, i. e., those which may be considered as drier metals and those which may be considered as non-driers. The first group or the driers includes lead, cobalt, manganese, iron, vanadium, and zinc. The second group or the non-driers includes those metals which have little or no drying effect. This group includes calcium, barium, strontium, magnesium, copper, nickel, chromium, and tin.

In selecting a metal for use in the preparation of either or both types of soaps required in our rust preventive composition, it is important that at least a portion of the total metal employed be a metal selected from the first group, i. e., having drying properties. The proportion of such metal to be employed will depend to a certain extent upon the activity of the metal selected in regard to its drying abilities. We have found that a rust

## 11

preventive composition in which lead was employed for producing all of the metal soaps is particularly desirable. In those cases in which manganese is the desired drying metal it is usually preferred to use at least an equal quantity of a metal selected from the second group such as calcium for example, and in those cases in which cobalt is the drying metal selected, it is well to use at least 2 parts of a non-drying metal soap to 1 part of the cobalt soap. Thus, as the drying effectiveness of the drier metal selected increases, the proportion of that metal used in the finished rust preventive should be decreased. In this connection it is generally understood that the effectiveness as a drier of 1 weight of cobalt is approximately equivalent to 8 weights of manganese and to 40 weights of lead.

*Finished rust preventive composition*

In preparing a finished rust preventive composition, we may simply combine the 50% thinner solutions of the two types of soaps, i. e., those of a semi-dry oil and those of synthetic acids, in the desired proportions and thus obtain a finished composition comprising about 50% by weight of a mixture of oil-soluble soaps and 50% by weight of thinner. To such a mixture we may add a small percentage of a cobalt drier as indicated above, and/or small percentages of lubricating oil and/or paraffin wax as desired. In compounding these ingredients it is essential that thorough mixing be employed to produce a homogeneous product. This compounding may be effected at ordinary atmospheric temperatures or at temperatures as high as 180° F. or 200° F.

We may, however, prefer to prepare both soaps without the addition of thinner to produce a solvent-free composition which may be subsequently diluted with thinner and in this case also, we may incorporate the cobalt drier, the paraffin wax and the lubricating oil in the solvent-free soap mixture by heating and agitating the mass, say at temperatures of 200° F. to about 300° F. to produce a homogeneous solvent-free mixture which may subsequently be thinned with a desired quantity of mineral solvent.

Examples of rust preventive compositions which we have found to be particularly effective as anti-corrosive agents when applied in thin films to metal surfaces are given below.

*Example I*

|                                                   | Per cent by weight |
|---------------------------------------------------|--------------------|
| Lead soap of tall oil                             | 40.0               |
| Lead soap of lubricating oil oxidate <sup>1</sup> | 15.0               |
| Petrolatum                                        | 5.0                |
| Cobalt drier (as metal)                           | 0.01               |
| Petroleum thinner                                 | 40.0               |

<sup>1</sup> An oxidate produced by oxidizing a highly solvent treated paraffinic Western lubricating oil having a Saybolt Universal viscosity of 50 seconds at 210° F., a V. I. of 99 and a V. G. C. of 0.805. This oil was oxidized by blowing with air at 270° F. for 36 hours under a pressure of 90 lbs./sq. in. gage and the resulting oxidate had an acid number of 53 mg. KOH/g. and a saponification number of 90 mg. KOH/g.

*Example II*

|                                                   | Per cent by weight |
|---------------------------------------------------|--------------------|
| Manganese soap of tall oil                        | 10.0               |
| Calcium soap of tall oil                          | 28.0               |
| Lead soap of lubricating oil oxidate <sup>1</sup> | 17.0               |
| Paraffin wax (122° F.-125° F. M. P.)              | 4.0                |
| Petroleum thinner                                 | 41.0               |

<sup>1</sup> This was the same lubricating oil oxidate as used in Example I.

## 12

*Example III*

|                                            | Per cent by weight |
|--------------------------------------------|--------------------|
| Lead soap of tall oil                      | 41.0               |
| Calcium soap of wax oxidate <sup>1</sup>   | 8.0                |
| Manganese soap of wax oxidate <sup>1</sup> | 4.0                |
| Barium sulfonate <sup>2</sup>              | 3.0                |
| Petroleum thinner                          | 44.0               |

<sup>1</sup> The wax oxidate was prepared by oxidizing paraffin wax (122° F. to 125° F. M. P.) for a period of 49 hours at 250° F. and at a pressure of 90 lbs./sq. in. gage. This oxidate had an acid number of 195 mg. KOH/g. and a saponification number of 345 mg. KOH/g.

<sup>2</sup> The barium salt of oil-soluble (mahogany) sulfonic acid.

*Example IV*

|                                         | Per cent by weight |
|-----------------------------------------|--------------------|
| Lead soap of rape seed oil              | 20.0               |
| Lead soap of tall oil                   | 15.0               |
| Lead soap of wax acids <sup>1</sup>     | 14.0               |
| Paraffin wax (122° F. to 125° F. M. P.) | 2.0                |
| Lubricating oil                         | 4.0                |
| Cobalt drier (as metal)                 | 0.01               |
| Petroleum thinner                       | 45.0               |

<sup>1</sup> The wax acids were obtained from the wax oxidate used in Example III by saponification with aqueous caustic and acidification of the thus formed calcium soaps with dilute mineral acid.

*Example V*

|                                     | Per cent by weight |
|-------------------------------------|--------------------|
| Lead soap of tall oil               | 39.0               |
| Lead soap of wax acids <sup>1</sup> | 13.0               |
| Sodium sulfonate <sup>2</sup>       | 4.0                |
| Petrolatum                          | 4.0                |
| Cobalt drier (as metal)             | 0.01               |
| Thinner                             | 40.0               |

<sup>1</sup> Wax acids as used in Example IV.

<sup>2</sup> The sodium salt of oil-soluble (mahogany) sulfonic acids.

*Example VI*

|                                       | Per cent by weight |
|---------------------------------------|--------------------|
| Cobalt soap of tall oil               | 5.0                |
| Calcium soap of tall oil              | 15.0               |
| Lead soap of tall oil                 | 20.0               |
| Lead soap of wax oxidate <sup>1</sup> | 17.0               |
| Lead sulfonate <sup>2</sup>           | 3.0                |
| Thinner                               | 40.0               |

<sup>1</sup> Wax oxidate as used in Example III.

<sup>2</sup> The lead salt of oil-soluble (mahogany) sulfonic acids.

The foregoing description and examples of our invention are not to be considered as limiting for many variations may be made by those skilled in the art without departing from the spirit or the scope of the following claims.

We claim:

1. An anti-rust composition comprising between about 5% and 95% by weight of an oil-soluble metal soap of a semi-drying oil, between about 3% and 85% by weight of an oil-soluble metal soap of synthetic organic acids produced by the liquid phase oxidation of a petroleum hydrocarbon, less than about 12% by weight of paraffin wax and less than about 12% by weight of lubricating oil.

2. An anti-rust composition comprising between about 5% and 95% by weight of an oil-soluble metal soap of a semi-drying oil, between about 3% and 85% by weight of an oil-soluble metal soap of synthetic organic acids produced by the liquid phase oxidation of a petroleum hydrocarbon and a small amount of an oil-soluble metal sulfonate.

3. An anti-rust composition comprising between about 5% and 95% by weight of an oil-soluble metal soap of a semi-drying oil, between about 3% and 85% by weight of an oil-soluble metal soap of synthetic organic acids produced

by the liquid phase oxidation of a petroleum hydrocarbon, a small amount of petrolatum and a small amount of a drier.

4. An anti-rust composition comprising between about 5% and 95% by weight of an oil-soluble metal soap of tall oil and between about 3% and 85% by weight of an oil-soluble metal soap of acids produced by the liquid phase oxidation of a highly paraffinic petroleum fraction.

5. An anti-rust composition comprising between about 5% and 95% by weight of an oil-soluble metal soap of tall oil, between about 3% and 85% by weight of an oil-soluble metal soap of acids produced by the liquid phase oxidation of a petroleum fraction, a small amount of an oil-soluble metal sulfonate, a small amount of paraffin wax and a drier.

6. An anti-rust composition as in claim 4 wherein said oil-soluble metal soaps are lead soaps.

7. An anti-rust composition comprising between about 5% and 95% by weight of an oil-soluble metal soap of a semi-drying oil and between about 3% and 85% by weight of an oil-soluble metal soap of synthetic organic acids produced by the liquid phase oxidation of a petroleum fraction wherein said oil-soluble metal soap of a semi-drying oil comprises a mixture of a drier metal soap and a non-drier metal soap of said semi-drying oil.

8. An anti-rust composition comprising between about 5% and 95% by weight of an oil-soluble metal soap of a semi-drying oil and between about 3% and 85% by weight of an oil-soluble metal soap of synthetic organic acids produced by the liquid phase oxidation of a petroleum fraction wherein said oil-soluble metal soap of synthetic organic acids comprises a mixture of a drier metal soap and a non-drier metal soap of said synthetic organic acids.

9. An anti-rust composition comprising between about 5% and about 95% by weight of an oil-soluble metal soap of a semi-drying oil, between about 3% and about 85% by weight of an oil-soluble metal soap of synthetic organic acids produced by the liquid phase oxidation of a highly paraffinic petroleum fraction, less than about 8% by weight of paraffin wax, less than about 8% by weight of lubricating oil and a drier, said drier being an oil-soluble salt of a metal selected from the class consisting of cobalt and manganese.

10. An anti-rust composition comprising between about 2.5% and about 47.5% by weight of an oil-soluble metal soap of a semi-drying oil, between about 1.5% and about 42.5% by weight of an oil-soluble metal soap of synthetic acids produced by oxidizing a hydrocarbon fraction, between about 1% and about 6% by weight of paraffin wax, between about 1% and about 6% by weight of lubricating oil, between about 0.01% and about 0.2% by weight of cobalt in the form of an oil-soluble cobalt salt and between about 30% and about 70% by weight of thinner.

11. An anti-rust composition comprising between about 25.0% and about 45.0% by weight of an oil-soluble metal soap of a semi-drying oil, between about 5.0% and about 20.0% by weight of an oil-soluble metal soap of synthetic acids produced by the liquid phase oxidation of a hydrocarbon fraction, between about 1.0% and about 5.0% by weight of an oil-soluble metal sulfonate, between about 1.0% and about 6.0% by weight of paraffin wax, between about 0.01% and about 0.1% by weight of cobalt in the form of an oil- 75

soluble cobalt salt and between about 30.0% and about 70.0% by weight of a thinner.

12. An anti-rust composition comprising about 40.0% by weight of lead tall oil soap, about 15.0% by weight of a lead soap of a lubricating oil oxidate, about 5.0% by weight of petrolatum, about 0.01% by weight of cobalt drier as metal and about 40.0% by weight of thinner, said oxidate being produced by oxidizing a highly solvent treated paraffinic Western lubricating oil.

13. An anti-rust composition comprising about 41.0% by weight of a lead soap of tall oil, about 8.0% by weight of a calcium soap of paraffin wax oxidate, about 4.0% by weight of a manganese soap of paraffin wax oxidate, about 3.0% by weight of a barium soap of oil-soluble sulfonic acid and about 44.0% by weight of a thinner.

14. An anti-rust composition comprising about 20.0% by weight of a lead soap of rape seed oil, about 15.0% by weight of a lead soap of tall oil, about 14.0% by weight of a lead soap of acids produced by oxidizing paraffin wax, about 2.0% by weight of paraffin wax, about 4.0% by weight of lubricating oil, about 0.01% by weight of cobalt drier as metal and about 45.0% by weight of thinner.

15. An anti-rust composition comprising between about 5% and 95% by weight of an oil-soluble metal soap of a semi-drying oil and between about 3% and 85% by weight of an oil-soluble metal soap of synthetic organic acids produced by the liquid phase oxidation of a petroleum hydrocarbon.

16. An anti-rust composition according to claim 15 wherein one of said oil-soluble metal soaps is a drier metal soap.

17. An anti-rust composition according to claim 15 wherein one of said oil-soluble metal soaps is a non-drier metal soap.

18. An anti-rust composition according to claim 7 wherein said drier metal is lead and said non-drier metal is calcium.

19. An anti-rust composition according to claim 7 wherein said drier metal is manganese and said non-drier metal is calcium.

20. An anti-rust composition according to claim 8 wherein said drier metal is lead and said non-drier metal is calcium.

21. An anti-rust composition according to claim 8 wherein said drier metal is manganese and said non-drier is calcium.

CHESTER E. WILSON.  
MARY LOUISE DODGE.

#### REFERENCES CITED

The following references are of record in the file of this patent:

#### UNITED STATES PATENTS

| Number    | Name                  | Date          |
|-----------|-----------------------|---------------|
| 2,348,715 | Adams et al.          | May 16, 1944  |
| 2,306,352 | Burrell               | Dec. 22, 1942 |
| 2,242,837 | Shields               | May 20, 1941  |
| 2,184,952 | Zimmer et al.         | Dec. 26, 1939 |
| 2,175,491 | Stresen-Reuter et al. | Oct. 10, 1939 |
| 1,630,101 | Wilkin                | May 24, 1927  |
| 1,364,134 | Morgan                | Jan. 4, 1921  |
| 2,266,325 | Lazar et al.          | Dec. 16, 1941 |
| 2,367,462 | Farber                | Jan. 16, 1945 |

#### FOREIGN PATENTS

| Number  | Country       | Date           |
|---------|---------------|----------------|
| 502,335 | Great Britain | Mar. 15, 1939  |
| 681,855 | Germany       | Oct. 3, 1939   |
| 111,339 | Australia     | Sept. 15, 1940 |